

## UNITED STATES PATENT OFFICE

2,208,161

## LUBRICATING COMPOSITION

Carl F. Prutton, Cleveland, Albert K. Smith, Shaker Heights, and Harry E. Johnson, Willoughby, Ohio, assignors, by mesne assignments, to The Lubri-Zol Development Corporation, Cleveland, Ohio, a corporation of Delaware

No Drawing. Application October 19, 1939,  
Serial No. 300,232

23 Claims. (Cl. 252—48)

This application is a continuation in part of our copending application Serial No. 170,501 filed October 22, 1937.

As disclosed in the patent of Carl F. Prutton No. 2,051,744, granted August 18, 1936, certain desirable improvements in the lubricating properties of lubricating oils may be secured by the combination therewith of certain halogenated organic compounds.

10 The use of sulphur for the purpose of imparting extreme pressure characteristics to lubricating compositions has been known for some time. It has been well recognized that in order for sulphur when used alone to impart extreme pressure characteristics to lubricating compositions it is necessary that such sulphur be present in active or corrosive form. It has been well known that certain organic compounds of sulphur contain sulphur in such stably bound condition that 15 when such compounds were added in minor amounts to a lubricating composition there was no appreciable increase in film strength.

We have discovered that by the combined use in a suitable oil base of certain halogenated organic compounds and organic sulphur compounds we are able to produce a lubricating composition superior in respect to those which have been available heretofore. The lubricating composition according to our invention is particularly applicable for use as an extreme pressure lubricant. The term "extreme pressure lubrication" is believed to be sufficiently well known to those familiar in the art that more particular definition thereof in this specification is unnecessary.

35 It is among the objects of our invention, therefore, to provide a lubricating composition which shall be superior to any which has heretofore been available.

Other objects of our invention will appear as the description proceeds.

To the accomplishment of the foregoing and related ends, said invention, then, consists of the means hereinafter fully described and particularly pointed out in the claims, the following description setting forth in detail one approved combination of ingredients embodying our invention, such disclosed means constituting,

however, but one of various forms in which the principle of the invention may be used.

Broadly stated, the improved lubricating compositions of our invention comprise the combination of a major proportion of lubricating oil, an organic halogen compound in a minor amount and a relatively inactive organic sulphur compound in an amount in which such sulphur compound would not substantially increase the extreme pressure characteristics of a plain mineral oil.

From the foregoing statement of our invention it will be observed that the lubricating compositions which comprise the same may be divided into three components, viz., the oil base, the halogen compound and the sulphur compound. These three components will first be considered separately and directions then given for the manner in which they may be blended in order to achieve the improved results.

20  
The oil base

The oil base of our lubricating compositions is a lubricating oil of the type best suited for the particular use for which the ultimate composition is designed. When the lubricating compositions of our invention are designed for the lubrication of automobiles, the oil base will of course preferably consist of a refined mineral lubricating oil of lubricating viscosity for the particular point of application. In other words, a conventional gear oil may be used for the lubrication of the gears and generally a lighter, more highly refined, oil will be used in the crank case.

This invention is applicable to lubricating compositions in which the base may consist either entirely or in part of synthetic oils, hydrogenated oils, and volatilized oils.

40 The oil base may also desirably contain other well known constituents such as those which improve the oiliness, pour point, cold test, and oxidation properties, etc., of the oil. In general, compositions of our invention may be employed with any commercially available addition agents for the above defined purposes since they are generally compatible with the same in the amounts 45 usually used.

*The halogen compounds*

The halogen compounds used should first be oil-soluble to the extent that the required amounts may be incorporated in the oil base in a stable form of true solution or colloidal suspension so that there will be no separation on storage, even over periods of considerable length and at reduced temperatures.

10 The halogen compound must be sufficiently non-volatile so that it will not be driven off from the lubricating composition during use. It will generally be found that the halogen compounds should have a vapor pressure less than atmospheric at a temperature of 140° C. and preferably at a temperature of 170° C.

15 The halogen compounds which may be employed as components of the composition may be divided into two broad classes, cyclic or ring compounds and aliphatic or chain compounds. In general, the ring compounds are more stable and less subject to hydrolysis than are the chain compounds particularly when the halogen is attached to a benzenoid ring structure. Therefore, where moisture and other conditions are encountered which tend to hydrolyze the halogen compounds, the ring compounds are generally preferable. The chain compounds are usually more active than the ring compounds and thus may be employed for the purpose of giving very high extreme pressure characteristics where such is necessary and where the conditions of use permit the employment of the relatively less stable chain compounds.

20 The class of oxygen and halogen bearing compounds will also be found to be of particular utility in our invention for reasons which may be generally stated as follows: The presence of the oxygen in the same molecule with the halogen tends to increase the tendency of the lubricating composition to be adsorbed on metallic surfaces and to activate the halogen so that the same are made more effective as extreme pressure addition agents. This is particularly true in the case where oxygen is added to the molecule of the 25 relatively stable halogenated carbon ring compounds which might otherwise be so stable as not to be sufficiently reactive with the bearing surfaces under conditions of extreme pressure. Examples of the various halogen bearing compounds which may thus be employed as one component of our composition are as follows:

A.—Aliphatic, such as halogenated:

## I.—Hydrocarbons, e. g.,

30 Hexachlorethane, and notably, those chlorinated or fluorinated hydrocarbons which contain from four to ten or more carbon atoms, e. g.

35 Chlorinated hexane  
Chlorinated octane  
Chlorinated decane  
Butylene dichloride  
Monochlorhexane  
1,2 dichlorhexane  
Amylene dichloride.

40 Other halogen substitution or addition products of commercial materials such as petroleum fractions including the paraffins, paraffin wax, foots oil, kerosene, mineral oil, etc.

## II.—Amines

45 Primary, secondary and tertiary, e. g.

Chlorinated or fluorinated, hexylamines, di-amylamines, tri-amylamines, such as:

5 Chlorinated tri-amyl amines  
Chlorinated tributyl amines  
Chlorinated hexyl amines

## III.—Nitriles, e. g.

Chlorinated or fluorinated:

10 Ethyl cyanide  
Butyl cyanide  
Octyl cyanide  
Lauryl nitrile  
Stearyl nitrile

## IV.—Sulphides, e. g.

15 Chlorinated or fluorinated:  
Di-ethyl sulphide  
Di-butyl sulphide  
Di-octyl sulphide  
Di-amyl sulphide  
Di-lauryl sulphide  
20 Di-cetyl sulphide

## V.—Mercaptans, e. g.

Chlorinated or fluorinated:  
Lauryl mercaptan  
Cetyl mercaptan  
Carnaubyl mercaptan  
Ceryl mercaptan  
Montanyl mercaptan  
Melissyl mercaptan  
Myricyl mercaptan  
30

## VI.—Thiocyanates (rhodanates) e. g.

Chlorinated or fluorinated:  
Ethyl thiocyanate  
Butyl thiocyanate  
Lauryl thiocyanate  
35 Cetyl thiocyanate  
Ceryl thiocyanate

## B.—Cyclic compounds, such as halogenated:

## I.—Benzene and related compounds such as:

## (1) Halogenated benzene, e. g.

(a) Chlorinated benzene, e. g.  
The dichlorbenzenes, notably the ortho compound

(b) Brominated benzene, e. g.  
Ortho-dibrom benzene

(c) Fluorinated benzene  
Cetyl thiocyanate

## (2) Halogenated derivatives of benzene such as:

(a) Halogenated homologs of benzene, e. g.

Mono-chlor toluene  
Mono-chlor xylene  
Mono-chlor cymene  
Ethyl mono-chlor benzenes  
55 Propyl mono-chlor benzenes  
Di-ethyl dichlor benzenes  
Propyl dichlor benzenes  
Di-ethyl tetrachlor benzenes

(b) Halogenated amino derivatives of benzene, e. g.

60 Chlorinated aniline  
Mono-chlor aniline (preferably the ortho-compound)  
Mono-chlor di-methyl aniline

Chlorinated toluidines  
Chlorinated xylydines

Chlorinated diphenylamine  
65 (c) Halogenated hydrobenzenes, e. g.

70 Hydrogenated dichlor-benzenes

Dichlorhexahydrobenzene  
(dichlor cyclohexane)

75

|                                                                            |                                                                                                                                                                                                                                                                                                                                                  |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|----------------------------------------------------------------------------|--------------------------------------------------------------------------------------------------------------------------------------------------------------------------------------------------------------------------------------------------------------------------------------------------------------------------------------------------|------------------------------------------------------|--|------------------------------------------------|-----------------------------------------------------------------|----|-----------------------------------------------------------------------------------------------------------------------------------------------|-----------------------------------------------------------------------------|-------------------------|--------------------------------------------------------------------------------------------------------------------------|-----------------------------------------------------------------------|-------------------------------------------------------|-----------------------------------------------------------------------------------------------------------------------------------|-----------------------------------------|-----------------------------------------------------------------|---------------------------------------------------------------|----------------------------------------|-----------------------------------------------------------------------|--------------|------------------------------------------------------------|-----------------------------------------------------------------|------------------------------------------------------|------------------------------------------|----------------------------------------|-----------------------------------------------------------------|--------------------------------|-----------------------------------------------------------------------------|--------------------------------------------------|-------------------------|----------------------------------|-----------------------------------------------------------------|----------------------------------------------------------------------------|-----------------------------------------|----------------------------------------|------------------------------------------------|----------------------------------------|-----------------------------------------------------------------------------|-----------------------------------------------------------------------------------------------------------------------------------------------|------------------------------------------------------------|--------------------------------------------------------------|--------------------------------------------------------------------------------------------------------------------------|------------------------------------------|-----------------------------------------|-----------------------------------------------------------------------------------------------------------------------------------|-----------------------------------------------------------------|----------------------------------------|-----------------------------------------------------------------------------|--------------------------------------------------|------------------------------------------------------------|-----------------------------------|----------------------------------------------------------------------------|------------------------------------------|-----------------------------------------|------------------------------------------------|--------------------------------|----------------------------------------|-----------------------------------------------------------------------------------------------------------------------------------------------|-------------------------|------------------------------------------------------------|--------------------------------------------------------------------------------------------------------------------------|----------------------------------------------------------------------------|------------------------------------------|-----------------------------------------------------------------------------------------------------------------------------------|--------------------------------------------------------------|--------------------------------|---------------------------------------------------------------|-----------------------------------------------------------------------------------------------------------------------------------------------|-------------------------|----------------------------------------|--------------------------------------------------------------------------------------------------------------------------|----------------------------------------------------------------------------|------------------------------------------------------------|-----------------------------------------------------------------------------------------------------------------------------------|------------------------------------------------|------------------------------------------|---------------------------------------------------------------|-----------------------------------------------------------------------------------------------------------------------------------------------|--------------------------------|------------------------------------------------------------|--------------------------------------------------------------------------------------------------------------------------|-------------------------|------------------------------------------|-----------------------------------------------------------------------------------------------------------------------------------|----------------------------------------------------------------------------|--------------------------------|---------------------------------------------------------------|------------------------------------------------|-------------------------|-------------------|-----------------------------------------------------------------------------------------------------------------------------------------------|----------------------------------------------------------------------------|-----------------------|--------------------------------------------------------------------------------------------------------------------------|------------------------------------------------|--------------------------------------------------------------|-----------------------------------------------------------------------------------------------------------------------------------|-----------------------------------------------------------------------------------------------------------------------------------------------|----------------|---------------------------------------------------------------|--------------------------------------------------------------------------------------------------------------------------|------------------|-------------------|--------------------------------------------------------------------------------------------------------------------------------------------------------------------------------------------------------------------------------------------------------------------------------------------------------------------------------------------------|--------------------------|-----------------------|---------------------------------------------------------------|---------------------|-------------------|-------------------|--------------------------------------------------------------|-----------------------|-------------------|----------------------|--------------------------------------------------------------|-----------------------|-------------------------|---------------|-------------------|-------------------|--------------------|-----------------------|--------------------|--------------------------------------------------------------|--------------------------------------------------------------|--------------------------|---------------------|--------------------|---------------------------|--------------------------|--------------------------------------------------------------|------------------------|----------------------|--------------------------|--------------------------------------------------------------------------------------------------------------------------------------------------------------------------------------------------------------------------------------------------------------------------------------------------------------------------------------------------|-------------------------|---------------------|--------------|-----------------------|--------------------------|------------------|--------------------|----------------------|--------------------------|--------------------------|-------------------------|---------------------|--------------------------------------------------------------|-------------------|--------------------------|------------------------|-----------------------|----------------------|--------------------------------------------------------------------------------------------------------------------------------------------------------------------------------------------------------------------------------------------------------------------------------------------------------------------------------------------------|--------------------------------------------------------------|-------------------------|--------------------------|---------------------------|--------------|---------------------|------------------------|--------------------|--------------------------|--------------------------------------------------------------------------------------------------------------------------------------------------------------------------------------------------------------------------------------------------------------------------------------------------------------------------------------------------|--------------------------|----------------------|---------------------|---------------------------|-------------------------|--------------------------|------------------------|--------------|----------------------|--------------------------------------------------------------------------------------------------------------------------------------------------------------------------------------------------------------------------------------------------------------------------------------------------------------------------------------------------|--------------------|-------------------------|--|--------------------------|--------------|--|---------------------------|--------------------|--|------------------------|--------------------------|----|--------------------------------------------------------------------------------------------------------------------------------------------------------------------------------------------------------------------------------------------------------------------------------------------------------------------------------------------------|---------------------------|----|--|------------------------|----|----|--------------------------------------------------------------------------------------------------------------------------------------------------------------------------------------------------------------------------------------------------------------------------------------------------------------------------------------------------|--|----|--|----|----|--|----|
| 5                                                                          | II.—Polyphenyls, and related compounds, including diphenyl, diphenyl benzenes, etc., such as                                                                                                                                                                                                                                                     |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| (1)                                                                        | Halogenated diphenyl, e. g.                                                                                                                                                                                                                                                                                                                      |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| (a)                                                                        | Chlorinated diphenyl, e. g.                                                                                                                                                                                                                                                                                                                      |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Mono-chlor diphenyls                                                                                                                                                                                                                                                                                                                             |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Dichlor diphenyls                                                                                                                                                                                                                                                                                                                                |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Tri-chlor diphenyls                                                                                                                                                                                                                                                                                                                              |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 10                                                                         | (b) Brominated diphenyl, e. g.                                                                                                                                                                                                                                                                                                                   |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | The mono-brom diphenyls                                                                                                                                                                                                                                                                                                                          |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| (c)                                                                        | Fluorinated diphenyl                                                                                                                                                                                                                                                                                                                             |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 15                                                                         | (2) Halogenated derivatives of diphenyl, such as,                                                                                                                                                                                                                                                                                                |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | (a) Halogenated homologs of diphenyl, e. g.                                                                                                                                                                                                                                                                                                      |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated phenyl-toluenes                                                                                                                                                                                                                                                                                                                      |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Ethylated, or propylated, chlorinated diphenyl, e. g.                                                                                                                                                                                                                                                                                            |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 20                                                                         | di-ethyl tetrachlor diphenyl                                                                                                                                                                                                                                                                                                                     |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | (b) Halogenated amino derivatives of diphenyl, e. g.                                                                                                                                                                                                                                                                                             |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated phenyl-anilines                                                                                                                                                                                                                                                                                                                      |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 25                                                                         | Chlorinated phenyl-toluidines                                                                                                                                                                                                                                                                                                                    |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated diphenyl amines                                                                                                                                                                                                                                                                                                                      |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated xenyl amines                                                                                                                                                                                                                                                                                                                         |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 30                                                                         | (c) Halogenated hydrodiphenyls, e. g.                                                                                                                                                                                                                                                                                                            |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated phenyl hexahydrobenzene                                                                                                                                                                                                                                                                                                              |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated dodecahydrodiphenyl                                                                                                                                                                                                                                                                                                                  |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 35                                                                         | III.—Naphthalene and related compounds, such as                                                                                                                                                                                                                                                                                                  |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| (1)                                                                        | Halogenated naphthalene                                                                                                                                                                                                                                                                                                                          |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| (a)                                                                        | Chlorinated naphthalene, e. g.                                                                                                                                                                                                                                                                                                                   |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | $\alpha$ -mono-chlor naphthalene                                                                                                                                                                                                                                                                                                                 |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 40                                                                         | (b)                                                                                                                                                                                                                                                                                                                                              | Brominated naphthalenes, e. g.                       |  |                                                | $\alpha$ -mono-brom naphthalene                                 |    | 45                                                                                                                                            | (c)                                                                         | Fluorinated naphthalene |                                                                                                                          |                                                                       | (2) Halogenated derivatives of naphthalenes, such as: |                                                                                                                                   |                                         | (a) Halogenated homologs of naphthalenes, e. g.                 |                                                               |                                        | Chlorinated methyl naphthalenes, such as $\alpha$ -methyl naphthalene |              | 50                                                         |                                                                 | Chlorinated ethyl, propyl, or isopropyl naphthalenes |                                          |                                        | (b) Halogenated amino derivatives of naphthalene, e. g.         |                                |                                                                             | Chlorinated naphthylamines                       |                         | 55                               |                                                                 | Mono-chlor naphthyl amine                                                  |                                         |                                        | (c) Halogenated hydronaphthalenes, e. g.       |                                        |                                                                             | Chlorinated decahydronaphthalene                                                                                                              |                                                            | 60                                                           |                                                                                                                          | Chlorinated tetrahydronaphthalene        |                                         | 65                                                                                                                                | IV.—Phenanthrene and anthracene and related compounds, such as: |                                        | (1)                                                                         | Chlorinated phenanthrene, chlorinated anthracene |                                                            | (2)                               | Halogenated derivatives of phenanthrene and anthracene such as:            |                                          |                                         | (a) Halogenated homologs, e. g.                |                                |                                        | Chlorinated 1-methyl phenanthrene                                                                                                             |                         | 70                                                         |                                                                                                                          | Chlorinated 3-methyl phenanthrene                                          |                                          | 75                                                                                                                                | Chlorinated 9,10 dimethyl phenanthrene                       |                                |                                                               | Chlorinated propyl and isopropyl derivatives of phenanthrene such as retene                                                                   | 5                       |                                        | Chlorinated dimethyl anthracenes                                                                                         |                                                                            |                                                            | Chlorinated $\alpha$ -methyl anthracene                                                                                           |                                                |                                          | Chlorinated $\beta$ -methyl anthracene                        | 10                                                                                                                                            |                                | Chlorinated propyl and isopropyl derivatives of anthracene |                                                                                                                          |                         | (b) Halogenated amino derivatives, e. g. | 15                                                                                                                                |                                                                            | Chlorinated phenanthryl amines |                                                               |                                                | Chlorinated anthramines |                   | 20                                                                                                                                            | (c) Halogenated hydrophenanthrenes and halogenated hydroanthracenes, e. g. | 20                    |                                                                                                                          | Chlorinated retene oil (contains hydro retene) |                                                              | 25                                                                                                                                | V.—Chrysene, picene, and related compounds, including their derivatives, such as homologs, amino derivatives and other substitution products. |                | 30                                                            | VI.—Bridged ring compounds, such as the terpenes and related compounds, and their derivatives, e. g. chlorinated pinene. | 30               | 35                | VII.—Heterocyclic compounds, such as pyridine, quinoline, pyrrole, thiophene, and derivatives of them, e. g. mono-chlor pyridine.                                                                                                                                                                                                                | 35                       | 40                    | VIII.—Nitriles derived from any of the above compounds, e. g. |                     |                   | Chlorinated:      |                                                              |                       | Benzonitrile      | 40                   |                                                              | Tolunitriles          |                         |               | Benzyl cyanide    |                   |                    | Naphthyl cyanide      |                    |                                                              | Xenyl cyanide                                                |                          |                     | Cyclohexyl cyanide |                           | 45                       | IX.—Sulphides derived from any of the above compounds, e. g. | 45                     |                      | Chlorinated:             |                                                                                                                                                                                                                                                                                                                                                  |                         | Diphenyl sulphide   |              |                       | Dibenzyl sulphide        | 50               |                    | Dixylyl sulphides    |                          |                          | Di-naphthyl sulphides   |                     |                                                              | Dixenyl sulphides |                          |                        | Dicyclohexyl sulphide |                      | 50                                                                                                                                                                                                                                                                                                                                               | X.—Mercaptans derived from any of the above compounds, e. g. | 55                      |                          | Chlorinated:              |              |                     | Benzyl mercaptan       |                    |                          | Phenyl benzyl mercaptans                                                                                                                                                                                                                                                                                                                         |                          |                      | Naphthyl mercaptans |                           |                         | Phenyl propyl mercaptans | 60                     |              | Cyclohexyl mercaptan |                                                                                                                                                                                                                                                                                                                                                  | 55                 | XI.—Thiocyanates, e. g. |  |                          | Chlorinated: |  |                           | Benzyl thiocyanate |  |                        | Phenyl ethyl thiocyanate | 65 |                                                                                                                                                                                                                                                                                                                                                  | Phenyl propyl thiocyanate |    |  | Cyclohexyl thiocyanate |    | 60 | It will be noted that the above enumerated examples of the organic ring compounds which are usually preferred when stability is a particularly desired characteristic are, in general, compounds of the aryl type, i. e., compounds containing benzoid ring structures and also of the type in which the halogen is directly attached to an atom |  | 65 |  | 70 | 70 |  | 75 |
| (b)                                                                        | Brominated naphthalenes, e. g.                                                                                                                                                                                                                                                                                                                   |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | $\alpha$ -mono-brom naphthalene                                                                                                                                                                                                                                                                                                                  |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 45                                                                         | (c)                                                                                                                                                                                                                                                                                                                                              | Fluorinated naphthalene                              |  |                                                | (2) Halogenated derivatives of naphthalenes, such as:           |    |                                                                                                                                               | (a) Halogenated homologs of naphthalenes, e. g.                             |                         |                                                                                                                          | Chlorinated methyl naphthalenes, such as $\alpha$ -methyl naphthalene |                                                       | 50                                                                                                                                |                                         | Chlorinated ethyl, propyl, or isopropyl naphthalenes            |                                                               |                                        | (b) Halogenated amino derivatives of naphthalene, e. g.               |              |                                                            | Chlorinated naphthylamines                                      |                                                      | 55                                       |                                        | Mono-chlor naphthyl amine                                       |                                |                                                                             | (c) Halogenated hydronaphthalenes, e. g.         |                         |                                  | Chlorinated decahydronaphthalene                                |                                                                            | 60                                      |                                        | Chlorinated tetrahydronaphthalene              |                                        | 65                                                                          | IV.—Phenanthrene and anthracene and related compounds, such as:                                                                               |                                                            | (1)                                                          | Chlorinated phenanthrene, chlorinated anthracene                                                                         |                                          | (2)                                     | Halogenated derivatives of phenanthrene and anthracene such as:                                                                   |                                                                 |                                        | (a) Halogenated homologs, e. g.                                             |                                                  |                                                            | Chlorinated 1-methyl phenanthrene |                                                                            | 70                                       |                                         | Chlorinated 3-methyl phenanthrene              |                                | 75                                     | Chlorinated 9,10 dimethyl phenanthrene                                                                                                        |                         |                                                            | Chlorinated propyl and isopropyl derivatives of phenanthrene such as retene                                              | 5                                                                          |                                          | Chlorinated dimethyl anthracenes                                                                                                  |                                                              |                                | Chlorinated $\alpha$ -methyl anthracene                       |                                                                                                                                               |                         | Chlorinated $\beta$ -methyl anthracene | 10                                                                                                                       |                                                                            | Chlorinated propyl and isopropyl derivatives of anthracene |                                                                                                                                   |                                                | (b) Halogenated amino derivatives, e. g. | 15                                                            |                                                                                                                                               | Chlorinated phenanthryl amines |                                                            |                                                                                                                          | Chlorinated anthramines |                                          | 20                                                                                                                                | (c) Halogenated hydrophenanthrenes and halogenated hydroanthracenes, e. g. | 20                             |                                                               | Chlorinated retene oil (contains hydro retene) |                         | 25                | V.—Chrysene, picene, and related compounds, including their derivatives, such as homologs, amino derivatives and other substitution products. |                                                                            | 30                    | VI.—Bridged ring compounds, such as the terpenes and related compounds, and their derivatives, e. g. chlorinated pinene. | 30                                             | 35                                                           | VII.—Heterocyclic compounds, such as pyridine, quinoline, pyrrole, thiophene, and derivatives of them, e. g. mono-chlor pyridine. | 35                                                                                                                                            | 40             | VIII.—Nitriles derived from any of the above compounds, e. g. |                                                                                                                          |                  | Chlorinated:      |                                                                                                                                                                                                                                                                                                                                                  |                          | Benzonitrile          | 40                                                            |                     | Tolunitriles      |                   |                                                              | Benzyl cyanide        |                   |                      | Naphthyl cyanide                                             |                       |                         | Xenyl cyanide |                   |                   | Cyclohexyl cyanide |                       | 45                 | IX.—Sulphides derived from any of the above compounds, e. g. | 45                                                           |                          | Chlorinated:        |                    |                           | Diphenyl sulphide        |                                                              |                        | Dibenzyl sulphide    | 50                       |                                                                                                                                                                                                                                                                                                                                                  | Dixylyl sulphides       |                     |              | Di-naphthyl sulphides |                          |                  | Dixenyl sulphides  |                      |                          | Dicyclohexyl sulphide    |                         | 50                  | X.—Mercaptans derived from any of the above compounds, e. g. | 55                |                          | Chlorinated:           |                       |                      | Benzyl mercaptan                                                                                                                                                                                                                                                                                                                                 |                                                              |                         | Phenyl benzyl mercaptans |                           |              | Naphthyl mercaptans |                        |                    | Phenyl propyl mercaptans | 60                                                                                                                                                                                                                                                                                                                                               |                          | Cyclohexyl mercaptan |                     | 55                        | XI.—Thiocyanates, e. g. |                          |                        | Chlorinated: |                      |                                                                                                                                                                                                                                                                                                                                                  | Benzyl thiocyanate |                         |  | Phenyl ethyl thiocyanate | 65           |  | Phenyl propyl thiocyanate |                    |  | Cyclohexyl thiocyanate |                          | 60 | It will be noted that the above enumerated examples of the organic ring compounds which are usually preferred when stability is a particularly desired characteristic are, in general, compounds of the aryl type, i. e., compounds containing benzoid ring structures and also of the type in which the halogen is directly attached to an atom |                           | 65 |  | 70                     | 70 |    | 75                                                                                                                                                                                                                                                                                                                                               |  |    |  |    |    |  |    |
| (c)                                                                        | Fluorinated naphthalene                                                                                                                                                                                                                                                                                                                          |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | (2) Halogenated derivatives of naphthalenes, such as:                                                                                                                                                                                                                                                                                            |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | (a) Halogenated homologs of naphthalenes, e. g.                                                                                                                                                                                                                                                                                                  |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated methyl naphthalenes, such as $\alpha$ -methyl naphthalene                                                                                                                                                                                                                                                                            |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 50                                                                         |                                                                                                                                                                                                                                                                                                                                                  | Chlorinated ethyl, propyl, or isopropyl naphthalenes |  |                                                | (b) Halogenated amino derivatives of naphthalene, e. g.         |    |                                                                                                                                               | Chlorinated naphthylamines                                                  |                         | 55                                                                                                                       |                                                                       | Mono-chlor naphthyl amine                             |                                                                                                                                   |                                         | (c) Halogenated hydronaphthalenes, e. g.                        |                                                               |                                        | Chlorinated decahydronaphthalene                                      |              | 60                                                         |                                                                 | Chlorinated tetrahydronaphthalene                    |                                          | 65                                     | IV.—Phenanthrene and anthracene and related compounds, such as: |                                | (1)                                                                         | Chlorinated phenanthrene, chlorinated anthracene |                         | (2)                              | Halogenated derivatives of phenanthrene and anthracene such as: |                                                                            |                                         | (a) Halogenated homologs, e. g.        |                                                |                                        | Chlorinated 1-methyl phenanthrene                                           |                                                                                                                                               | 70                                                         |                                                              | Chlorinated 3-methyl phenanthrene                                                                                        |                                          | 75                                      | Chlorinated 9,10 dimethyl phenanthrene                                                                                            |                                                                 |                                        | Chlorinated propyl and isopropyl derivatives of phenanthrene such as retene | 5                                                |                                                            | Chlorinated dimethyl anthracenes  |                                                                            |                                          | Chlorinated $\alpha$ -methyl anthracene |                                                |                                | Chlorinated $\beta$ -methyl anthracene | 10                                                                                                                                            |                         | Chlorinated propyl and isopropyl derivatives of anthracene |                                                                                                                          |                                                                            | (b) Halogenated amino derivatives, e. g. | 15                                                                                                                                |                                                              | Chlorinated phenanthryl amines |                                                               |                                                                                                                                               | Chlorinated anthramines |                                        | 20                                                                                                                       | (c) Halogenated hydrophenanthrenes and halogenated hydroanthracenes, e. g. | 20                                                         |                                                                                                                                   | Chlorinated retene oil (contains hydro retene) |                                          | 25                                                            | V.—Chrysene, picene, and related compounds, including their derivatives, such as homologs, amino derivatives and other substitution products. |                                | 30                                                         | VI.—Bridged ring compounds, such as the terpenes and related compounds, and their derivatives, e. g. chlorinated pinene. | 30                      | 35                                       | VII.—Heterocyclic compounds, such as pyridine, quinoline, pyrrole, thiophene, and derivatives of them, e. g. mono-chlor pyridine. | 35                                                                         | 40                             | VIII.—Nitriles derived from any of the above compounds, e. g. |                                                |                         | Chlorinated:      |                                                                                                                                               |                                                                            | Benzonitrile          | 40                                                                                                                       |                                                | Tolunitriles                                                 |                                                                                                                                   |                                                                                                                                               | Benzyl cyanide |                                                               |                                                                                                                          | Naphthyl cyanide |                   |                                                                                                                                                                                                                                                                                                                                                  | Xenyl cyanide            |                       |                                                               | Cyclohexyl cyanide  |                   | 45                | IX.—Sulphides derived from any of the above compounds, e. g. | 45                    |                   | Chlorinated:         |                                                              |                       | Diphenyl sulphide       |               |                   | Dibenzyl sulphide | 50                 |                       | Dixylyl sulphides  |                                                              |                                                              | Di-naphthyl sulphides    |                     |                    | Dixenyl sulphides         |                          |                                                              | Dicyclohexyl sulphide  |                      | 50                       | X.—Mercaptans derived from any of the above compounds, e. g.                                                                                                                                                                                                                                                                                     | 55                      |                     | Chlorinated: |                       |                          | Benzyl mercaptan |                    |                      | Phenyl benzyl mercaptans |                          |                         | Naphthyl mercaptans |                                                              |                   | Phenyl propyl mercaptans | 60                     |                       | Cyclohexyl mercaptan |                                                                                                                                                                                                                                                                                                                                                  | 55                                                           | XI.—Thiocyanates, e. g. |                          |                           | Chlorinated: |                     |                        | Benzyl thiocyanate |                          |                                                                                                                                                                                                                                                                                                                                                  | Phenyl ethyl thiocyanate | 65                   |                     | Phenyl propyl thiocyanate |                         |                          | Cyclohexyl thiocyanate |              | 60                   | It will be noted that the above enumerated examples of the organic ring compounds which are usually preferred when stability is a particularly desired characteristic are, in general, compounds of the aryl type, i. e., compounds containing benzoid ring structures and also of the type in which the halogen is directly attached to an atom |                    | 65                      |  | 70                       | 70           |  | 75                        |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated ethyl, propyl, or isopropyl naphthalenes                                                                                                                                                                                                                                                                                             |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | (b) Halogenated amino derivatives of naphthalene, e. g.                                                                                                                                                                                                                                                                                          |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated naphthylamines                                                                                                                                                                                                                                                                                                                       |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 55                                                                         |                                                                                                                                                                                                                                                                                                                                                  | Mono-chlor naphthyl amine                            |  |                                                | (c) Halogenated hydronaphthalenes, e. g.                        |    |                                                                                                                                               | Chlorinated decahydronaphthalene                                            |                         | 60                                                                                                                       |                                                                       | Chlorinated tetrahydronaphthalene                     |                                                                                                                                   | 65                                      | IV.—Phenanthrene and anthracene and related compounds, such as: |                                                               | (1)                                    | Chlorinated phenanthrene, chlorinated anthracene                      |              | (2)                                                        | Halogenated derivatives of phenanthrene and anthracene such as: |                                                      |                                          | (a) Halogenated homologs, e. g.        |                                                                 |                                | Chlorinated 1-methyl phenanthrene                                           |                                                  | 70                      |                                  | Chlorinated 3-methyl phenanthrene                               |                                                                            | 75                                      | Chlorinated 9,10 dimethyl phenanthrene |                                                |                                        | Chlorinated propyl and isopropyl derivatives of phenanthrene such as retene | 5                                                                                                                                             |                                                            | Chlorinated dimethyl anthracenes                             |                                                                                                                          |                                          | Chlorinated $\alpha$ -methyl anthracene |                                                                                                                                   |                                                                 | Chlorinated $\beta$ -methyl anthracene | 10                                                                          |                                                  | Chlorinated propyl and isopropyl derivatives of anthracene |                                   |                                                                            | (b) Halogenated amino derivatives, e. g. | 15                                      |                                                | Chlorinated phenanthryl amines |                                        |                                                                                                                                               | Chlorinated anthramines |                                                            | 20                                                                                                                       | (c) Halogenated hydrophenanthrenes and halogenated hydroanthracenes, e. g. | 20                                       |                                                                                                                                   | Chlorinated retene oil (contains hydro retene)               |                                | 25                                                            | V.—Chrysene, picene, and related compounds, including their derivatives, such as homologs, amino derivatives and other substitution products. |                         | 30                                     | VI.—Bridged ring compounds, such as the terpenes and related compounds, and their derivatives, e. g. chlorinated pinene. | 30                                                                         | 35                                                         | VII.—Heterocyclic compounds, such as pyridine, quinoline, pyrrole, thiophene, and derivatives of them, e. g. mono-chlor pyridine. | 35                                             | 40                                       | VIII.—Nitriles derived from any of the above compounds, e. g. |                                                                                                                                               |                                | Chlorinated:                                               |                                                                                                                          |                         | Benzonitrile                             | 40                                                                                                                                |                                                                            | Tolunitriles                   |                                                               |                                                | Benzyl cyanide          |                   |                                                                                                                                               | Naphthyl cyanide                                                           |                       |                                                                                                                          | Xenyl cyanide                                  |                                                              |                                                                                                                                   | Cyclohexyl cyanide                                                                                                                            |                | 45                                                            | IX.—Sulphides derived from any of the above compounds, e. g.                                                             | 45               |                   | Chlorinated:                                                                                                                                                                                                                                                                                                                                     |                          |                       | Diphenyl sulphide                                             |                     |                   | Dibenzyl sulphide | 50                                                           |                       | Dixylyl sulphides |                      |                                                              | Di-naphthyl sulphides |                         |               | Dixenyl sulphides |                   |                    | Dicyclohexyl sulphide |                    | 50                                                           | X.—Mercaptans derived from any of the above compounds, e. g. | 55                       |                     | Chlorinated:       |                           |                          | Benzyl mercaptan                                             |                        |                      | Phenyl benzyl mercaptans |                                                                                                                                                                                                                                                                                                                                                  |                         | Naphthyl mercaptans |              |                       | Phenyl propyl mercaptans | 60               |                    | Cyclohexyl mercaptan |                          | 55                       | XI.—Thiocyanates, e. g. |                     |                                                              | Chlorinated:      |                          |                        | Benzyl thiocyanate    |                      |                                                                                                                                                                                                                                                                                                                                                  | Phenyl ethyl thiocyanate                                     | 65                      |                          | Phenyl propyl thiocyanate |              |                     | Cyclohexyl thiocyanate |                    | 60                       | It will be noted that the above enumerated examples of the organic ring compounds which are usually preferred when stability is a particularly desired characteristic are, in general, compounds of the aryl type, i. e., compounds containing benzoid ring structures and also of the type in which the halogen is directly attached to an atom |                          | 65                   |                     | 70                        | 70                      |                          | 75                     |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Mono-chlor naphthyl amine                                                                                                                                                                                                                                                                                                                        |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | (c) Halogenated hydronaphthalenes, e. g.                                                                                                                                                                                                                                                                                                         |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated decahydronaphthalene                                                                                                                                                                                                                                                                                                                 |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 60                                                                         |                                                                                                                                                                                                                                                                                                                                                  | Chlorinated tetrahydronaphthalene                    |  | 65                                             | IV.—Phenanthrene and anthracene and related compounds, such as: |    | (1)                                                                                                                                           | Chlorinated phenanthrene, chlorinated anthracene                            |                         | (2)                                                                                                                      | Halogenated derivatives of phenanthrene and anthracene such as:       |                                                       |                                                                                                                                   | (a) Halogenated homologs, e. g.         |                                                                 |                                                               | Chlorinated 1-methyl phenanthrene      |                                                                       | 70           |                                                            | Chlorinated 3-methyl phenanthrene                               |                                                      | 75                                       | Chlorinated 9,10 dimethyl phenanthrene |                                                                 |                                | Chlorinated propyl and isopropyl derivatives of phenanthrene such as retene | 5                                                |                         | Chlorinated dimethyl anthracenes |                                                                 |                                                                            | Chlorinated $\alpha$ -methyl anthracene |                                        |                                                | Chlorinated $\beta$ -methyl anthracene | 10                                                                          |                                                                                                                                               | Chlorinated propyl and isopropyl derivatives of anthracene |                                                              |                                                                                                                          | (b) Halogenated amino derivatives, e. g. | 15                                      |                                                                                                                                   | Chlorinated phenanthryl amines                                  |                                        |                                                                             | Chlorinated anthramines                          |                                                            | 20                                | (c) Halogenated hydrophenanthrenes and halogenated hydroanthracenes, e. g. | 20                                       |                                         | Chlorinated retene oil (contains hydro retene) |                                | 25                                     | V.—Chrysene, picene, and related compounds, including their derivatives, such as homologs, amino derivatives and other substitution products. |                         | 30                                                         | VI.—Bridged ring compounds, such as the terpenes and related compounds, and their derivatives, e. g. chlorinated pinene. | 30                                                                         | 35                                       | VII.—Heterocyclic compounds, such as pyridine, quinoline, pyrrole, thiophene, and derivatives of them, e. g. mono-chlor pyridine. | 35                                                           | 40                             | VIII.—Nitriles derived from any of the above compounds, e. g. |                                                                                                                                               |                         | Chlorinated:                           |                                                                                                                          |                                                                            | Benzonitrile                                               | 40                                                                                                                                |                                                | Tolunitriles                             |                                                               |                                                                                                                                               | Benzyl cyanide                 |                                                            |                                                                                                                          | Naphthyl cyanide        |                                          |                                                                                                                                   | Xenyl cyanide                                                              |                                |                                                               | Cyclohexyl cyanide                             |                         | 45                | IX.—Sulphides derived from any of the above compounds, e. g.                                                                                  | 45                                                                         |                       | Chlorinated:                                                                                                             |                                                |                                                              | Diphenyl sulphide                                                                                                                 |                                                                                                                                               |                | Dibenzyl sulphide                                             | 50                                                                                                                       |                  | Dixylyl sulphides |                                                                                                                                                                                                                                                                                                                                                  |                          | Di-naphthyl sulphides |                                                               |                     | Dixenyl sulphides |                   |                                                              | Dicyclohexyl sulphide |                   | 50                   | X.—Mercaptans derived from any of the above compounds, e. g. | 55                    |                         | Chlorinated:  |                   |                   | Benzyl mercaptan   |                       |                    | Phenyl benzyl mercaptans                                     |                                                              |                          | Naphthyl mercaptans |                    |                           | Phenyl propyl mercaptans | 60                                                           |                        | Cyclohexyl mercaptan |                          | 55                                                                                                                                                                                                                                                                                                                                               | XI.—Thiocyanates, e. g. |                     |              | Chlorinated:          |                          |                  | Benzyl thiocyanate |                      |                          | Phenyl ethyl thiocyanate | 65                      |                     | Phenyl propyl thiocyanate                                    |                   |                          | Cyclohexyl thiocyanate |                       | 60                   | It will be noted that the above enumerated examples of the organic ring compounds which are usually preferred when stability is a particularly desired characteristic are, in general, compounds of the aryl type, i. e., compounds containing benzoid ring structures and also of the type in which the halogen is directly attached to an atom |                                                              | 65                      |                          | 70                        | 70           |                     | 75                     |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated tetrahydronaphthalene                                                                                                                                                                                                                                                                                                                |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 65                                                                         | IV.—Phenanthrene and anthracene and related compounds, such as:                                                                                                                                                                                                                                                                                  |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| (1)                                                                        | Chlorinated phenanthrene, chlorinated anthracene                                                                                                                                                                                                                                                                                                 |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| (2)                                                                        | Halogenated derivatives of phenanthrene and anthracene such as:                                                                                                                                                                                                                                                                                  |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | (a) Halogenated homologs, e. g.                                                                                                                                                                                                                                                                                                                  |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated 1-methyl phenanthrene                                                                                                                                                                                                                                                                                                                |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 70                                                                         |                                                                                                                                                                                                                                                                                                                                                  | Chlorinated 3-methyl phenanthrene                    |  | 75                                             | Chlorinated 9,10 dimethyl phenanthrene                          |    |                                                                                                                                               | Chlorinated propyl and isopropyl derivatives of phenanthrene such as retene | 5                       |                                                                                                                          | Chlorinated dimethyl anthracenes                                      |                                                       |                                                                                                                                   | Chlorinated $\alpha$ -methyl anthracene |                                                                 |                                                               | Chlorinated $\beta$ -methyl anthracene | 10                                                                    |              | Chlorinated propyl and isopropyl derivatives of anthracene |                                                                 |                                                      | (b) Halogenated amino derivatives, e. g. | 15                                     |                                                                 | Chlorinated phenanthryl amines |                                                                             |                                                  | Chlorinated anthramines |                                  | 20                                                              | (c) Halogenated hydrophenanthrenes and halogenated hydroanthracenes, e. g. | 20                                      |                                        | Chlorinated retene oil (contains hydro retene) |                                        | 25                                                                          | V.—Chrysene, picene, and related compounds, including their derivatives, such as homologs, amino derivatives and other substitution products. |                                                            | 30                                                           | VI.—Bridged ring compounds, such as the terpenes and related compounds, and their derivatives, e. g. chlorinated pinene. | 30                                       | 35                                      | VII.—Heterocyclic compounds, such as pyridine, quinoline, pyrrole, thiophene, and derivatives of them, e. g. mono-chlor pyridine. | 35                                                              | 40                                     | VIII.—Nitriles derived from any of the above compounds, e. g.               |                                                  |                                                            | Chlorinated:                      |                                                                            |                                          | Benzonitrile                            | 40                                             |                                | Tolunitriles                           |                                                                                                                                               |                         | Benzyl cyanide                                             |                                                                                                                          |                                                                            | Naphthyl cyanide                         |                                                                                                                                   |                                                              | Xenyl cyanide                  |                                                               |                                                                                                                                               | Cyclohexyl cyanide      |                                        | 45                                                                                                                       | IX.—Sulphides derived from any of the above compounds, e. g.               | 45                                                         |                                                                                                                                   | Chlorinated:                                   |                                          |                                                               | Diphenyl sulphide                                                                                                                             |                                |                                                            | Dibenzyl sulphide                                                                                                        | 50                      |                                          | Dixylyl sulphides                                                                                                                 |                                                                            |                                | Di-naphthyl sulphides                                         |                                                |                         | Dixenyl sulphides |                                                                                                                                               |                                                                            | Dicyclohexyl sulphide |                                                                                                                          | 50                                             | X.—Mercaptans derived from any of the above compounds, e. g. | 55                                                                                                                                |                                                                                                                                               | Chlorinated:   |                                                               |                                                                                                                          | Benzyl mercaptan |                   |                                                                                                                                                                                                                                                                                                                                                  | Phenyl benzyl mercaptans |                       |                                                               | Naphthyl mercaptans |                   |                   | Phenyl propyl mercaptans                                     | 60                    |                   | Cyclohexyl mercaptan |                                                              | 55                    | XI.—Thiocyanates, e. g. |               |                   | Chlorinated:      |                    |                       | Benzyl thiocyanate |                                                              |                                                              | Phenyl ethyl thiocyanate | 65                  |                    | Phenyl propyl thiocyanate |                          |                                                              | Cyclohexyl thiocyanate |                      | 60                       | It will be noted that the above enumerated examples of the organic ring compounds which are usually preferred when stability is a particularly desired characteristic are, in general, compounds of the aryl type, i. e., compounds containing benzoid ring structures and also of the type in which the halogen is directly attached to an atom |                         | 65                  |              | 70                    | 70                       |                  | 75                 |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated 3-methyl phenanthrene                                                                                                                                                                                                                                                                                                                |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 75                                                                         | Chlorinated 9,10 dimethyl phenanthrene                                                                                                                                                                                                                                                                                                           |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated propyl and isopropyl derivatives of phenanthrene such as retene                                                                                                                                                                                                                                                                      | 5                                                    |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated dimethyl anthracenes                                                                                                                                                                                                                                                                                                                 |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated $\alpha$ -methyl anthracene                                                                                                                                                                                                                                                                                                          |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated $\beta$ -methyl anthracene                                                                                                                                                                                                                                                                                                           | 10                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated propyl and isopropyl derivatives of anthracene                                                                                                                                                                                                                                                                                       |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | (b) Halogenated amino derivatives, e. g.                                                                                                                                                                                                                                                                                                         | 15                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated phenanthryl amines                                                                                                                                                                                                                                                                                                                   |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated anthramines                                                                                                                                                                                                                                                                                                                          |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 20                                                                         | (c) Halogenated hydrophenanthrenes and halogenated hydroanthracenes, e. g.                                                                                                                                                                                                                                                                       | 20                                                   |  | Chlorinated retene oil (contains hydro retene) |                                                                 | 25 | V.—Chrysene, picene, and related compounds, including their derivatives, such as homologs, amino derivatives and other substitution products. |                                                                             | 30                      | VI.—Bridged ring compounds, such as the terpenes and related compounds, and their derivatives, e. g. chlorinated pinene. | 30                                                                    | 35                                                    | VII.—Heterocyclic compounds, such as pyridine, quinoline, pyrrole, thiophene, and derivatives of them, e. g. mono-chlor pyridine. | 35                                      | 40                                                              | VIII.—Nitriles derived from any of the above compounds, e. g. |                                        |                                                                       | Chlorinated: |                                                            |                                                                 | Benzonitrile                                         | 40                                       |                                        | Tolunitriles                                                    |                                |                                                                             | Benzyl cyanide                                   |                         |                                  | Naphthyl cyanide                                                |                                                                            |                                         | Xenyl cyanide                          |                                                |                                        | Cyclohexyl cyanide                                                          |                                                                                                                                               | 45                                                         | IX.—Sulphides derived from any of the above compounds, e. g. | 45                                                                                                                       |                                          | Chlorinated:                            |                                                                                                                                   |                                                                 | Diphenyl sulphide                      |                                                                             |                                                  | Dibenzyl sulphide                                          | 50                                |                                                                            | Dixylyl sulphides                        |                                         |                                                | Di-naphthyl sulphides          |                                        |                                                                                                                                               | Dixenyl sulphides       |                                                            |                                                                                                                          | Dicyclohexyl sulphide                                                      |                                          | 50                                                                                                                                | X.—Mercaptans derived from any of the above compounds, e. g. | 55                             |                                                               | Chlorinated:                                                                                                                                  |                         |                                        | Benzyl mercaptan                                                                                                         |                                                                            |                                                            | Phenyl benzyl mercaptans                                                                                                          |                                                |                                          | Naphthyl mercaptans                                           |                                                                                                                                               |                                | Phenyl propyl mercaptans                                   | 60                                                                                                                       |                         | Cyclohexyl mercaptan                     |                                                                                                                                   | 55                                                                         | XI.—Thiocyanates, e. g.        |                                                               |                                                | Chlorinated:            |                   |                                                                                                                                               | Benzyl thiocyanate                                                         |                       |                                                                                                                          | Phenyl ethyl thiocyanate                       | 65                                                           |                                                                                                                                   | Phenyl propyl thiocyanate                                                                                                                     |                |                                                               | Cyclohexyl thiocyanate                                                                                                   |                  | 60                | It will be noted that the above enumerated examples of the organic ring compounds which are usually preferred when stability is a particularly desired characteristic are, in general, compounds of the aryl type, i. e., compounds containing benzoid ring structures and also of the type in which the halogen is directly attached to an atom |                          | 65                    |                                                               | 70                  | 70                |                   | 75                                                           |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| (c) Halogenated hydrophenanthrenes and halogenated hydroanthracenes, e. g. | 20                                                                                                                                                                                                                                                                                                                                               |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated retene oil (contains hydro retene)                                                                                                                                                                                                                                                                                                   |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 25                                                                         | V.—Chrysene, picene, and related compounds, including their derivatives, such as homologs, amino derivatives and other substitution products.                                                                                                                                                                                                    |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 30                                                                         | VI.—Bridged ring compounds, such as the terpenes and related compounds, and their derivatives, e. g. chlorinated pinene.                                                                                                                                                                                                                         | 30                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 35                                                                         | VII.—Heterocyclic compounds, such as pyridine, quinoline, pyrrole, thiophene, and derivatives of them, e. g. mono-chlor pyridine.                                                                                                                                                                                                                | 35                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 40                                                                         | VIII.—Nitriles derived from any of the above compounds, e. g.                                                                                                                                                                                                                                                                                    |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated:                                                                                                                                                                                                                                                                                                                                     |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Benzonitrile                                                                                                                                                                                                                                                                                                                                     | 40                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Tolunitriles                                                                                                                                                                                                                                                                                                                                     |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Benzyl cyanide                                                                                                                                                                                                                                                                                                                                   |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Naphthyl cyanide                                                                                                                                                                                                                                                                                                                                 |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Xenyl cyanide                                                                                                                                                                                                                                                                                                                                    |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Cyclohexyl cyanide                                                                                                                                                                                                                                                                                                                               |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 45                                                                         | IX.—Sulphides derived from any of the above compounds, e. g.                                                                                                                                                                                                                                                                                     | 45                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated:                                                                                                                                                                                                                                                                                                                                     |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Diphenyl sulphide                                                                                                                                                                                                                                                                                                                                |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Dibenzyl sulphide                                                                                                                                                                                                                                                                                                                                | 50                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Dixylyl sulphides                                                                                                                                                                                                                                                                                                                                |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Di-naphthyl sulphides                                                                                                                                                                                                                                                                                                                            |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Dixenyl sulphides                                                                                                                                                                                                                                                                                                                                |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Dicyclohexyl sulphide                                                                                                                                                                                                                                                                                                                            |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 50                                                                         | X.—Mercaptans derived from any of the above compounds, e. g.                                                                                                                                                                                                                                                                                     | 55                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated:                                                                                                                                                                                                                                                                                                                                     |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Benzyl mercaptan                                                                                                                                                                                                                                                                                                                                 |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Phenyl benzyl mercaptans                                                                                                                                                                                                                                                                                                                         |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Naphthyl mercaptans                                                                                                                                                                                                                                                                                                                              |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Phenyl propyl mercaptans                                                                                                                                                                                                                                                                                                                         | 60                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Cyclohexyl mercaptan                                                                                                                                                                                                                                                                                                                             |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 55                                                                         | XI.—Thiocyanates, e. g.                                                                                                                                                                                                                                                                                                                          |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Chlorinated:                                                                                                                                                                                                                                                                                                                                     |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Benzyl thiocyanate                                                                                                                                                                                                                                                                                                                               |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Phenyl ethyl thiocyanate                                                                                                                                                                                                                                                                                                                         | 65                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Phenyl propyl thiocyanate                                                                                                                                                                                                                                                                                                                        |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
|                                                                            | Cyclohexyl thiocyanate                                                                                                                                                                                                                                                                                                                           |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 60                                                                         | It will be noted that the above enumerated examples of the organic ring compounds which are usually preferred when stability is a particularly desired characteristic are, in general, compounds of the aryl type, i. e., compounds containing benzoid ring structures and also of the type in which the halogen is directly attached to an atom |                                                      |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 65                                                                         |                                                                                                                                                                                                                                                                                                                                                  | 70                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |
| 70                                                                         |                                                                                                                                                                                                                                                                                                                                                  | 75                                                   |  |                                                |                                                                 |    |                                                                                                                                               |                                                                             |                         |                                                                                                                          |                                                                       |                                                       |                                                                                                                                   |                                         |                                                                 |                                                               |                                        |                                                                       |              |                                                            |                                                                 |                                                      |                                          |                                        |                                                                 |                                |                                                                             |                                                  |                         |                                  |                                                                 |                                                                            |                                         |                                        |                                                |                                        |                                                                             |                                                                                                                                               |                                                            |                                                              |                                                                                                                          |                                          |                                         |                                                                                                                                   |                                                                 |                                        |                                                                             |                                                  |                                                            |                                   |                                                                            |                                          |                                         |                                                |                                |                                        |                                                                                                                                               |                         |                                                            |                                                                                                                          |                                                                            |                                          |                                                                                                                                   |                                                              |                                |                                                               |                                                                                                                                               |                         |                                        |                                                                                                                          |                                                                            |                                                            |                                                                                                                                   |                                                |                                          |                                                               |                                                                                                                                               |                                |                                                            |                                                                                                                          |                         |                                          |                                                                                                                                   |                                                                            |                                |                                                               |                                                |                         |                   |                                                                                                                                               |                                                                            |                       |                                                                                                                          |                                                |                                                              |                                                                                                                                   |                                                                                                                                               |                |                                                               |                                                                                                                          |                  |                   |                                                                                                                                                                                                                                                                                                                                                  |                          |                       |                                                               |                     |                   |                   |                                                              |                       |                   |                      |                                                              |                       |                         |               |                   |                   |                    |                       |                    |                                                              |                                                              |                          |                     |                    |                           |                          |                                                              |                        |                      |                          |                                                                                                                                                                                                                                                                                                                                                  |                         |                     |              |                       |                          |                  |                    |                      |                          |                          |                         |                     |                                                              |                   |                          |                        |                       |                      |                                                                                                                                                                                                                                                                                                                                                  |                                                              |                         |                          |                           |              |                     |                        |                    |                          |                                                                                                                                                                                                                                                                                                                                                  |                          |                      |                     |                           |                         |                          |                        |              |                      |                                                                                                                                                                                                                                                                                                                                                  |                    |                         |  |                          |              |  |                           |                    |  |                        |                          |    |                                                                                                                                                                                                                                                                                                                                                  |                           |    |  |                        |    |    |                                                                                                                                                                                                                                                                                                                                                  |  |    |  |    |    |  |    |

which is a part of such ring structure. Very satisfactory results may be obtained when two or more different halogens are present in the same molecule, ortho brom chlor benzene being a good example of such a compound. If the aromatic compounds have been alkylated, they are often especially effective.

Especially good results are generally secured when the halogen in the composition is present in the form of an oxygen containing or bearing organic ring compound. This class of addition agents has the desirable property of increased oiliness stability as compared with the chain compounds generally, and at the same time a sufficient amount of activity so as to impart the necessary properties to the ultimate composition.

The oxygen and halogen containing or bearing organic ring compounds, above referred to, may be classified as follows, viz:

- I. "Carbon ring" type compounds
- Of the aromatic, or allied type, including derivatives of benzene, naphthalene, anthracene, etc., also compounds of the bridged ring type, such as the terpenes, and related compounds.
  - Of the class including the cycloparaffins, cyclo-olefines, etc. Examples of this class are derivatives of the following:
    - Hydrogenation products of benzene (e. g. cyclohexane, cyclohexene, cyclohexadiene).
    - Hydrogenation products of naphthalene (e. g. decahydro-naphthalene, tetrahydro-naphthalene, etc.).
    - Naphthenes, naphthenic acid, etc.
    - Of mixed type such as derivatives of indene, hydrindene, hydranthracene, etc.

- II. "Heterogeneous ring" type compounds
- Of the aromatic or allied type including derivatives of pyridine, quinoline, etc.
  - Other types such as furan and its derivatives and derivatives of triphene, pyrrole, etc.

The foregoing compounds may also be classified according to the nature of the attachment of the oxygen to the compound, viz:

- I'. Directly attached to one or more carbon atoms, as in the case of:
- Ethers and analogous compounds
  - Compounds containing the  $\equiv C-OH$  radicle, such as alcohols and other derivatives of carbinol (including phenols, cresols, naphthols, etc.)
  - Compounds containing the carbonyl ( $=C=O$ ) radicle, such as aldehydes, ketones, quinones, (e. g., anthra quinone) acids, esters and salts of organic acids, thio-acids and esters of thio-acids.
  - Compounds in which oxygen forms a part of the ring structure, e. g., furan and its derivatives, etc.
  - Compounds with an inorganic radicle where the oxygen is directly attached to a carbon atom
- Arsenate  
Hypochlorite  
Phosphite  
Thiophosphate  
Thiophosphite  
B-hydroxylamines

II'. Indirectly attached through the means of some other atom, i. e., in the form of an inorganic radicle, e. g.:

|                         |    |
|-------------------------|----|
| Arsenate                | 5  |
| Chlorate                | 10 |
| Chlorite                | 10 |
| Cyanate                 | 10 |
| $\alpha$ -hydroxylamine | 10 |
| Nitrate                 | 15 |
| Nitrite                 | 15 |
| Nitro                   | 15 |
| Nitroso                 | 15 |
| Oxime                   | 15 |
| Perchlorate             | 15 |
| Phosphate               | 15 |
| Sulphate                | 20 |
| Sulphite                | 20 |
| Sulphinic acid          | 20 |
| Sulphone                | 20 |
| Sulphonic acid          | 20 |
| Sulphoxide              | 20 |
| Thio-sulphate           | 20 |

In addition to the substituents containing oxygen, other substituents may also be present without destroying, and in certain cases improving, the effect on the lubricating qualities of the oil such as other aryl groups, alkyl groups, and amino and substituted amino groups, imino, azo, hydrazo, hydrozine, nitrile, mercapto, sulphide, polysulphide.

Specific examples of compounds of the various classes of halogen and oxygen containing ring compounds are listed in the co-pending application of Carl F. Prutton, Ser. No. 737,070 filed July 26, 1934.

This second component of the composition, i. e., that which supplied halogen, will, for certain purposes, desirably be in the form of a halogen and oxygen bearing organic compound. While it is preferable to have both oxygen and halogen present in the same molecule when employing this type of second component of our composition, desirable results may nevertheless be effected by the combined use as the second component of the composition of a halogen bearing organic ring compound which does not contain oxygen with a separate organic oxygen compound. Such separate organic oxygen compound may be any of the organic ring compounds listed in said application, Ser. No. 737,070 as being the ones from which halogen derivatives may be prepared and in addition any similar organic oxygen compounds which do not contain ring structures, for example, alkyl, allyl, etc., alcohols, ethers, aldehydes, ketones, acids, esters and salts. Of these compounds the carboxylic acids and the esters and salts of such acids are preferred, e. g., fatty oils, vegetable oils, oleic acid, stearic acid, amyl acetate, butyl stearate, dibutyl phthalate, methyl salicylate, naphthenic acid, butyl naphthenate; sodium, calcium and aluminum stearates and oleates; sodium, calcium and lead naphthenates.

#### The organic sulphur compounds

As previously indicated, the third component of our composition is sulphur in the form of a relatively inactive organic sulphur compound in an amount in which such sulphur compound would not substantially increase the extreme pressure characteristics of a plain mineral oil.

In other words, our invention comprises the combined use of a halogen compound and relatively inactive sulphur to the end that the cooperation between the second and third components of our composition results in the achievement of a film strength in the resultant composition which is due to the cooperation between such second and third components. In other words, the organic sulphur compound is of the type or present in amounts such that it, when used alone without the halogen, does not substantially increase the film strength of plain mineral oil but which, when used in conjunction with a halogen compound, is activated by the latter to the production of an unexpected result flowing from the cooperative effect of the second and third components of our composition.

While there is no generally accepted standard machine or test procedure in universal use to-day for the purpose of determining extreme pressure characteristics of a lubricating composition, nevertheless there are a number of machines available to-day which are currently being used with fairly uniform and satisfactory results. The well-known Almen machine was employed in making determinations referred to herein. When in our specification and claims we refer to the fact that the sulphur compound is of the type or present in such amounts as to not substantially increase the extreme pressure characteristics of a plain mineral oil, we mean such characteristics as would be determined by the use of either the Timken or Almen machine under the conditions of test prescribed by the manufacturers of such machines.

The effect of sulphur compounds in increasing film strength is enormously enhanced by the presence of halogen-containing, or of halogen- and oxygen-containing, organic compounds, especially if the relative proportions of such sulphur and halogen compounds are within certain ranges. Sulphur compounds in amounts which have a negligible effect in increasing film strength when used by themselves are very effective when used in combination with the proper proportion of halogen-bearing organic compounds. Organic sulphides, disulphides, mercaptans, mercaptoles, thio-acids, and their esters, dithio-acids, and their esters, sulphones, sulphoxides, sulphonic acids, and their esters, sulphinic acids, and their esters, sulphone amides, sulphone chlorides, thio-amides, thio-anilides, organic thiocyanates, organic xanthates etc., (which may or may not contain a ring structure) are examples of sulphur compounds which act in this way. The table below shows the results obtained when solutions in mineral oil of such compounds, along and with halogen compounds such as chlorinated paraffin wax and chlorinated diphenyl ether, were tested on an Almen lubricant testing machine. The chlorinated wax contained about 40% of chlorine and had been treated to remove free chlorine and hydrogen chloride. The chlorinated diphenyl ether contained a total of about 45% chlorine with about 10% chlorine in the form of addition products, and had been treated with quick-lime at a temperature of about 90° C. The increase in film strength of the oil caused by compounds dissolved in it is shown, and is stated in terms of additional pounds of weight applied to the loading arm of the machine re-

quired to cause breakdown, as compared with the oil alone.

| Percent of dibenzyl disulphide                                                | 'Percent of chlorinated wax | Average increase in breakdown load           | 5  |
|-------------------------------------------------------------------------------|-----------------------------|----------------------------------------------|----|
| 0                                                                             | 4                           | 8                                            |    |
| 0                                                                             | 8                           | 12                                           |    |
| 1                                                                             | 0                           | 1                                            |    |
| 2                                                                             | 0                           | 2                                            |    |
| 1                                                                             | 4                           | More than 24                                 | 10 |
| 2                                                                             | 8                           | More than 24                                 |    |
| <i>Percent of benzyl thiocyanate</i>                                          |                             |                                              |    |
| 0.5                                                                           | 0                           | 2                                            |    |
| 0.5                                                                           | 4                           | More than 24                                 |    |
| <i>Percent of diphenyl sulphide</i>                                           |                             | <i>Percent of chlorinated diphenyl ether</i> | 15 |
| 0                                                                             | 1                           | 6                                            |    |
| 0                                                                             | 2                           | 8                                            |    |
| 0                                                                             | 4                           | 9                                            |    |
| 0.5                                                                           | 0                           | 0                                            |    |
| 2.9                                                                           | 0                           | 0                                            |    |
| 5.8                                                                           | 0                           | 2                                            | 20 |
| 0.5                                                                           | 1                           | 10                                           |    |
| 2.9                                                                           | 2                           | 14                                           |    |
| 5.8                                                                           | 4                           | 22                                           |    |
| <i>Percent of diphenyl disulphide</i>                                         |                             |                                              | 25 |
| 2                                                                             | 0                           | 4                                            |    |
| 2                                                                             | 1                           | 22                                           |    |
| <i>Percent of dibenzyl disulphide</i>                                         |                             |                                              |    |
| 1½                                                                            | 3                           | More than 24                                 |    |
| 3                                                                             | 0                           | 4                                            |    |
| 3                                                                             | 1½                          | More than 24                                 |    |
| <i>Percent of amyl mercaptan</i>                                              |                             |                                              | 30 |
| 1.5                                                                           | 0                           | 0                                            |    |
| 1.5                                                                           | 3                           | More than 24                                 |    |
| <i>Percent of dilauryl sulphide</i>                                           |                             |                                              |    |
| 0.5                                                                           | 0                           | 3                                            |    |
| 0.5                                                                           | 4                           | More than 24                                 |    |
| <i>Percent of dibutyl disulphide</i>                                          |                             |                                              | 35 |
| 0.5                                                                           | 0                           | 4                                            |    |
| 0.5                                                                           | 0.5                         | 14                                           |    |
| <i>Percent of product of reaction of butylene diamine with CS<sub>2</sub></i> |                             |                                              |    |
| 3                                                                             | 0                           | 4                                            |    |
| 3                                                                             | 3                           | More than 24                                 | 40 |
| <i>Percent di-methylbenzyl sulphide*</i>                                      |                             |                                              |    |
| ½                                                                             | 0                           | 3                                            |    |
| ½                                                                             | 1½                          | More than 24                                 |    |

\*This material was an impure product containing about 10 per cent total sulphur and about 3 per cent total chlorine, the latter in non-hydrolyzable form. It was prepared by chlorinating boiling xylene until the boiling point reached 200° C. and allowing the chlorinated xylene to react with sodium sulphide in alcoholic solution. The product separated as a heavier oily layer and was treated with calcium oxide at 100° C.

Following is a list of additional specific examples of organic sulphur compounds which have been found satisfactory for use:

|                                                                         |    |
|-------------------------------------------------------------------------|----|
| Tallow mercaptan (the reaction product of chlorinated tallow with NaHS) | 55 |
| Tri-o-cresyl thiophosphate                                              |    |
| Di (di-isobutylene) disulphide                                          |    |
| Dibutyl sulphide                                                        |    |
| Di-amyl sulphide                                                        |    |
| Di-amyl disulphide                                                      | 60 |
| Dihydroxy diphenyl disulphide                                           |    |
| Alkylated hydroxy phenyl disulphides                                    |    |
| Lauryl thiocyanate                                                      |    |
| Benzyl ester of xanthic acid                                            |    |

For other specific examples of organic sulphur compounds which may thus be employed as the third component of the composition of our invention, reference may be had to the list of organic sulphur compounds contained in the copending application of Carl F. Prutton, Ser. No. 193,960 filed March 4, 1938.

In order to protect bearings, gears, etc. from very severe overloads, it is sometimes advisable to use a halogen-containing compound which is so unstable as to be appreciably corrosive under 75

normal conditions. Since chain compounds are generally more corrosive, i. e. more unstable than ring compounds, they are admirably suited for this purpose. In these circumstances the corrosive effect of such chain compounds and of halogenated organic ring compounds of the addition type for example, may be greatly inhibited by the addition of certain other oil-soluble compounds, such as (1) organic bases, aromatic and alkyl amines, triethanolamine, quinoline, etc., (2) organic phosphates, e. g., tri-butyl phosphate, tri-phenyl phosphate, tri-cresyl phosphate, etc. Also certain of the halogen and sulphur compounds referred to above have similar corrosion-inhibiting effects, notably, (1) the phosphates of chlorinated ring compounds, e. g. tri-chlorophenyl phosphate, (2) mercaptans and chlor-mercaptans. For other specific examples of corrosion inhibitors reference may be had to copending applications, Ser. Nos. 119,132; 297,872; 297,873; 297,874; 297,875 and 297,876.

#### Percentages and proportions

25 The percentages and proportions within which the three components of our improved lubricating compositions are employed will depend largely upon the purpose for which the lubricating composition is designed and the character of the 30 three components themselves.

In general, the addition agents which are added to the lubricating oil base should have a vapor pressure less than atmospheric at the temperatures to which the finished product is subjected 35 either during storage or use. For the lubrication of ice machines, one type of addition agent would be suitable which however might be entirely unsuited for the lubrication of internal combustion engines operating at extremely high temperatures. In general, the addition agents which 40 comprise the second and third components of our composition should have a vapor pressure less than atmospheric at 140° C. and preferably at 170° C.

45 The second component of our composition, i. e. the halogen bearing compound will be employed in percentages which are dictated by the results desired and the type of oil base and sulphur compound with which they are combined, etc. For most purposes, the halogen bearing compounds will be employed in percentages less than 50 20% of the total composition. In most cases, amounts less than 10% will be employed and for certain uses such as for crank case oils in internal combustion engines, amounts less than 5% will be employed. In general, the halogen bearing compound will be required to be present in amounts in excess of .02% in order to be effective. The ranges of percentages which may be given therefore for the amount of halogen bearing organic compound which is employed 55 may be given as from about .02% to about 20%; from about .1% to about 10% and from about .5% to about 5%.

60 When a separate organic oxygen compound is employed in combination with a halogen bearing organic compound as the second component of our composition, such oxygen compound will generally be employed in amounts from about .10% to about 10%.

65 The organic sulphur compounds employed as the third component of our composition will generally be employed in the range of from about .01% to about 20%. For most uses, this range 70 will be from about .01% to about 10%, the range 75

of from about .05% to about 5% being usually preferred.

Especially good results are secured when the halogen compound employed is selected from the general class which contains from about 25% to about 50% of halogen. With this class of halogen compounds optimum results will be secured in high-temperature lubricants by the employment of from one-tenth to 2% of the halogenated compounds. 10

As above indicated, optimum results are secured by maintaining a certain proportional relationship between the second and third components depending upon the relative activity of these components. Thus for example, with a 15 relatively very inactive sulphur compound and a relatively very active halogen compound the proportional relationship would be in the range of one part of the sulphur compound to one part of the halogen compound. With the sulphur 20 compound relatively less inactive and the halogen compound of relatively low activity, the proportional relationship would be in the range of one part of the sulphur compound to about ten parts of the halogen compound. Intermediate 25 ranges which have been successfully employed have been one part of sulphur compound to five parts of halogen compound and one part of sulphur compound to two parts of halogen compound. For the most part good results will be 30 obtained with a proportional relationship of about one part of sulphur compound to three parts of halogen compound.

Other modes of applying the principle of our invention may be employed instead of the one 35 explained, change being made as regards the materials employed in carrying out the process, provided the ingredient or ingredients stated in any of the following claims or the equivalent of such stated ingredient or ingredients be employed. 40

We therefore particularly point out and distinctly claim as our invention:

1. A lubricating composition comprising the combination of a major proportion of mineral oil, a relatively inactive organic sulphur compound in an amount in which such sulphur compound would not substantially increase the extreme pressure characteristics of a plain mineral oil, and a minor amount of an organic halogen compound. 45

2. A lubricating composition comprising the combination of a major proportion of mineral oil, a relatively inactive organic sulphur compound in an amount in which such sulphur compound would not substantially increase the extreme pressure characteristics of a plain mineral oil, and a minor amount of an aromatic halogen compound. 55

3. A lubricating composition comprising the combination of a major proportion of mineral oil, a relatively inactive organic sulphur compound in an amount in which such sulphur compound would not substantially increase the extreme pressure characteristics of a plain mineral oil, and a minor amount of an aliphatic halogen compound. 60

4. A lubricating composition comprising the combination of a major proportion of mineral oil, a relatively inactive organic sulphur compound of the class consisting of aliphatic sulphides and aliphatic polysulphides in an amount in which such sulphur compound would not substantially increase the extreme pressure characteristics of a plain mineral oil, and a minor amount of an organic halogen compound. 70

5. A lubricating composition comprising the combination of a major proportion of mineral oil, an organic disulphide in an amount in which such compound would not substantially increase the extreme pressure characteristics of a plain mineral oil, and a minor amount of an organic halogen compound. 5
10. A lubricating composition comprising the combination of a major proportion of mineral oil, dibenzyl disulphide in an amount in which such compound would not substantially increase the extreme pressure characteristics of a plain mineral oil, and a minor amount of an organic halogen compound. 10
15. 7. A lubricating composition comprising the combination of a major proportion of mineral oil, a relatively inactive organic sulphur compound in an amount in which such sulphur compound would not substantially increase the extreme pressure characteristics of a plain mineral oil, and a minor amount of a halogen-bearing petroleum derivative. 15
20. 8. A lubricating composition comprising the combination of a major proportion of mineral oil, a relatively inactive organic sulphur compound in an amount in which such sulphur compound would not substantially increase the extreme pressure characteristics of a plain mineral oil, and a minor amount of a halogenated petroleum wax. 20
25. 9. A lubricating composition comprising the combination of a major proportion of mineral oil, a relatively inactive organic sulphur compound in an amount in which such sulphur compound would not substantially increase the extreme pressure characteristics of a plain mineral oil, and a minor amount of a halogenated mineral oil. 25
30. 10. A lubricating composition comprising the combination of a major proportion of mineral oil, a relatively inactive organic sulphur compound in an amount in which such sulphur compound would not substantially increase the extreme pressure characteristics of a plain mineral oil, and a minor amount of a halogenated foot oil. 30
35. 11. A lubricating composition comprising the combination of a major proportion of mineral oil, a relatively inactive organic sulphur compound of the class consisting of sulphides and polysulphides in an amount in which such sulphur compound would not substantially increase the extreme pressure characteristics of a plain mineral oil, and a minor amount of a halogenated petroleum fraction. 35
40. 12. A lubricating composition comprising the combination of a major proportion of mineral oil, a relatively inactive organic sulphur compound of the class consisting of sulphides and polysulphides in an amount in which such sulphur compound would not substantially increase the extreme pressure characteristics of a plain mineral oil, and a minor amount of a chlorinated paraffin wax. 40
45. 13. A lubricating composition comprising a major proportion of mineral oil, a relatively inactive organic sulphur compound in an amount in which such sulphur compound would not substantially increase the extreme pressure characteristics of a plain mineral oil, and from about 0.10% to about 10% of an organic halogen compound having a vapor pressure less than atmospheric at a temperature of 140° C. 45
50. 14. A lubricating composition comprising a major proportion of mineral oil, a relatively in- 50
55. active organic sulphur compound in an amount in which such sulphur compound would not substantially increase the extreme pressure characteristics of a plain mineral oil, and from about 0.10% to about 10% of an aromatic halogen compound having a vapor pressure less than atmospheric at a temperature of 140° C. 5
60. 15. A lubricating composition comprising a major proportion of mineral oil, a relatively inactive organic sulphur compound in an amount in which such sulphur compound would not substantially increase the extreme pressure characteristics of a plain mineral oil, and from about 0.10% to about 10% of an aliphatic halogen compound having a vapor pressure less than atmospheric at a temperature of 140° C. 10
65. 16. A lubricating composition comprising a major proportion of mineral oil, a relatively inactive organic sulphur compound in an amount in which such sulphur compound would not substantially increase the extreme pressure characteristics of a plain mineral oil, and from about 0.50% to about 5% of an organic halogen compound having a vapor pressure less than atmospheric at a temperature of 170° C. 20
70. 17. A lubricating composition comprising a major proportion of mineral oil, a relatively inactive organic sulphur compound in an amount in which such sulphur compound would not substantially increase the extreme pressure characteristics of a plain mineral oil, and from about 0.10% to about 10% of a halogen bearing petroleum derivative having a vapor pressure less than atmospheric at a temperature of 140° C. 30
75. 18. A lubricating composition comprising a major proportion of mineral oil, a relatively inactive organic sulphur compound of the class consisting of aromatic sulphides and aromatic polysulphides in an amount in which such sulphur compound would not substantially increase the extreme pressure characteristics of a plain mineral oil, and a minor amount of a halogen bearing petroleum derivative having a vapor pressure less than atmospheric at a temperature of 140° C. 40
80. 19. A lubricating composition comprising a major proportion of mineral oil, an organic polysulphide in an amount in which such sulphur compound would not substantially increase the extreme pressure characteristics of a plain mineral oil, and a minor amount of a halogen bearing petroleum derivative having a vapor pressure less than atmospheric at a temperature of 140° C. 50
85. 20. A lubricating composition comprising a major proportion of mineral oil, an aromatic polysulphide in an amount in which such sulphur compound would not substantially increase the extreme pressure characteristics of a plain mineral oil, and a minor amount of a halogen bearing petroleum derivative having a vapor pressure less than atmospheric at a temperature of 140° C. 60
90. 21. A lubricating composition comprising a major proportion of mineral oil, an organic disulphide in an amount in which such sulphur compound would not substantially increase the extreme pressure characteristics of a plain mineral oil, and a minor amount of a halogen bearing petroleum derivative having a vapor pressure less than atmospheric at a temperature of 140° C. 65
95. 22. A lubricating composition comprising a major proportion of mineral oil, an aromatic disulphide in an amount in which such sulphur compound would not substantially increase the extreme pressure characteristics of a plain min- 70
100. 75

eral oil, and a minor amount of a halogen bearing petroleum derivative having a vapor pressure less than atmospheric at a temperature of 140° C.

23. A lubricating composition comprising a major proportion of mineral oil, dibenzyl disulphide in an amount in which such sulphur compound would not substantially increase the ex-

treme pressure characteristics of a plain mineral oil, and a minor amount of a halogen bearing petroleum derivative having a vapor pressure less than atmospheric at a temperature of 140° C.

CARL F. PRUITTON. 5  
ALBERT K. SMITH.  
HARRY E. JOHNSON.